

Nov. 6, 1923.

1,472,956

E. N. BIEGLER

BUILDING CONSTRUCTION

Filed Dec. 12, 1921

Fig. 1.



Fig. 2.



Witness:

F. G. Johnson

Inventor:

Edward N. Biegler

By Crommell, Gist, Brown & Atches

## UNITED STATES PATENT OFFICE.

EDWARD N. BIEGLER, OF CHICAGO, ILLINOIS.

## BUILDING CONSTRUCTION.

Application filed December 12, 1921. Serial No. 521,623.

*To all whom it may concern:*

Be it known that I, EDWARD N. BIEGLER, a citizen of the United States, residing at Chicago, in the county of Cook and State of Illinois, have invented certain new and useful Improvements in Building Constructions, of which the following is a specification.

This invention relates generally to building constructions, and particularly to improvements in the structure of elements designed for use in building structures, such as portions of floors, walls, ceilings, roofs or the like. The invention contemplates the embodiment of the structure hereinafter described not only as integral portions of the parts of building structures above mentioned, but also as separate members or articles of manufacture formed particularly for use in such employment, such as tile.

The general object of the invention is the provision of a construction for use in the above mentioned portions of building which may be made of substantially moisture proof or non-absorptive materials and therefore possesses distinct advantages for use as sanitary and waterproof wall or floor covering, and which at the same time possesses characteristics of strength, resiliency and non-combustibility which render it particularly advantageous in the contemplated uses.

Another object of the invention is the provision of such a construction which is very light and at the same time very strong, whereby it is adapted for extensive use in building construction without imposing an undesirable load upon the supporting parts of the structure.

A more particular object of the invention is the production of an improved form of tile or surface finish element which is designed to be manufactured in quantity in a factory and subsequently installed in place in a building construction, said tile having certain characteristics of structure which particularly adapt it for firm and immovable mounting in the intended location.

Other and further objects of the invention will be pointed out hereinafter, indicated in the appended claims, or obvious upon an understanding of the invention from the following disclosure.

For the purpose of the present application I have disclosed herein one form in which the invention may be embodied, namely, in the form of a tile; but it is to be understood

that this is here presented for illustrative purposes merely, and that it is not intended as exhaustive of all forms which the invention may take structurally. Therefore, the present illustrative disclosure is not to be construed as limiting the invention as claimed, short of its true and most comprehensive scope in the art.

In the drawings, forming a part of this specification I have illustrated in Fig. 1 a sectional view of a tile supported in a suitable mounting and embodying the features of my invention; and

Fig. 2 is a top view of a tile showing the arrangement of reinforcing members therein as contemplated in my invention.

The nature of the invention will be best understood by reference to these drawings in detail, from which it will be understood that the numeral 1 designates any suitable supporting foundation, such as a floor portion, wall portion or roof portion of a building. Upon this foundation is imposed a cementitious coating 2 of plastic material, suitably held in place upon the foundation and adapted in turn to support the surfacing portions of the structure. These surfacing portions, in the form illustrated, comprise a number or series of flat tile suitably laid together to afford the desired finish. These tile comprise a combination including a cushion or under-coating designated by the numeral 4, the composition of which will be described hereinafter. This cushion or under-coating may be formed in situ, or it may be formed in a mould when the tile is manufactured in a factory and afterwards installed.

Disposed at the lower portion of this cushion or under-coating is a series of reinforcing elements designated by the numeral 5, and here illustrated as being formed of expanded metal lath of the type customarily employed in building construction. These reinforcing elements extend across the tile, but not entirely to the edge thereof, so that they are substantially completely enclosed within the plastic material, excepting at the bottom or rear surface of the tile. At the rear surface of the tile certain portions of these reinforcing elements may be left protruding a sufficient distance to form anchoring means whereby it may be retained in the plastic scratch-coating 2. In the customary formation of the element, as where it is formed as a tile in a

suitable form of mould, the reinforcing elements 5 are customarily placed in the bottom of the form, and then the plastic composition, designated by the numeral 4, is poured over them and pressed down about them. As a result of this fashion of forming the tile, the flow of the plastic material will be limited to some extent by the reinforcing elements 5, with the result that 5 below certain of the elements 5 the back surface of the tile will be indented or pitted by a number of void spaces, herein designated by the numeral 4<sup>a</sup>. After the under-coating 4 has thus been formed to the proper 10 thickness, a series of upper reinforcing elements 6 is disposed on the top of the under-coating, while it is still in a plastic condition. These reinforcing elements 6 preferably extend across the tile in a direction 15 transverse of the direction of the major axis of the reinforcing elements 5. Moreover the upper elements 6 are spaced apart from the lower elements 5 an appreciable distance by the material of the under-coating 25 4. After the upper reinforcing elements 6 are placed in position, they are covered by a top or surfacing coat 7 of a suitable plastic material such as the composition hereinafter described. This surfacing coat is applied while the cushion coat 4 is still soft, and by suitable pressure is thoroughly packed upon the same and about the projecting portions of the upper reinforcing elements 6. The surface 30 35 of the coating 7 is then given the desired finish and the material is allowed to set. I find it advantageous to form the surface coating 7 of about one-half the thickness of the cushion coating, so that the relation 40 is about one-third to two-thirds with respect to the entire thickness of the structure. When a tile of this construction is imposed upon the plastic cementitious scratch coating 2, and pressed thereupon, 45 a certain amount of the material of the latter will be forced into the voids or pits 4<sup>a</sup> at the rear surface of the tile, and when the scratch coating 2 sets, this connection of the two will operate effectively as a lock 50 to retain the tile or surfacing element 55 against detachment or movement upon the foundation 1. It will be observed that this lock arrangement permits the material of the scratch coating to penetrate the tile into the vicinity of the reinforcing elements.

I will now describe in detail one composition which may be employed in formation of the structure just described, which 60 composition constitutes an essential part of my invention. This composition has the characteristics of possessing great strength when combined with the reinforcing elements in the manner above described, and at the same time is comparatively light, water-

proof, sanitary, fireproof, resilient, and possessed of a peculiar quality which renders it particularly comfortable underfoot. In the preparation of this composition I first 70 prepare a mixture of dry powdered ingredients as follows: calcined magnesite approximately 33½%; pulverized slate stone approximately 10%; silica approximately 10%; pulverized cork approximately 20%; asbestos fibre approximately 5%; kieselguhr 75 approximately 2%; coloring matter, such as oxide of iron approximately 8 to 10% and the balance wood flour of a fineness suitable for the particular part of the structure, as hereinafter specified. These several ingredients combined in the proportion by weight above mentioned, are suitably mixed together and then combined with the liquid ingredients which previously have been 80 mixed together as follows: A magnesium chloride solution reduced with water to a density of approximately 20° Baumé, to which is added a mixture of silicate of soda and crude oil in proportion of approximately 85 ten per cent. The proportion of silicate of soda to crude oil may vary as desired. A sufficient quantity of this liquid mixture is combined with the dry powder constituent 90 to form a plastic mortar, which is placed in the mould or deposited upon the lower 95 reinforcing members 5 and coating 2, in any suitable fashion and smoothed off to the desired thickness. The wood flour employed in forming this lower or cushion coat may be and preferably is relatively coarse, as 100 sawdust. The wood flour employed in the surface coating 7 however should be very finely pulverized. Another feature which distinguishes the top surface coat 4 from the surface coat 7 is the employment of coloring 105 matter in the latter to give the tile the desired decorative effect. Obviously it is not necessary to employ this coloring matter in the under coating. The metallic reinforcing elements 5 and 6 are given a waterproofing coating before they are incorporated in the structure. A suitable coating for preparing and protecting the reinforcing elements against corrosion is 110 one formed by dissolving gilsonite or asphalt in a suitable hydrocarbon solvent such as naphtha or benzol. The metal reinforcing elements are dipped in this material before their insertion into the structure, and thereby are given a waterproofing coating which protects them from moisture and which aids in the adhesion of the plastic material to the elements.

A distinct advantage presented by a 115 structure as above described is its ability to resist warping influences, particularly influences which might tend to make the surface cup. This results not only from the nature of the composition forming the body 120 of the structure, but also from the com-

bination of body material of this type with reinforcing elements in the manner specified. The construction moreover accomplishes a very great reduction in weight from that of the customary tile construction. This is accomplished not only by the reduction in the weight of the material which goes to form the surface elements, such as the tile above described, but also in the reduction of the backing or mounting for such surfacing elements. In ordinary tile construction it is necessary to form the backing, corresponding to applicant's scratch coat 2, of very substantial thickness, in order to resist cracking. The construction of applicant's structure, however, enables it effectively to resist cracking, so that cracks which may occur in the scratch coating are not transmitted into the surfacing elements. Moreover, where the scratch coating is formed of my above described composition, it is less subject to cracking, and may be used effectively in much thinner coats and is of much less weight per unit of volume than the cements ordinarily employed. By the employment of my improved construction a reduction of weight per unit of surface may be obtained amounting to substantially 70%.

While I have described above one composition of which the articles herein claimed may be formed, it is to be understood that they may be constructed of other suitable plastic materials. Furthermore, while the particular composition herein described is not herein claimed, such omission to claim the subject-matter of the composition is not to be regarded as an abandonment or dedication of the same, as I purpose to claim such composition in a co-pending application.

I claim:

1. An article of the class described comprising the combination of a cushion coating of rigid material having reinforcing elements embedded adjacent its rear surface, a surface coating imposed upon said cushion coating and consolidated therewith, reinforcing elements embedded at the junction of said coatings, and the cushion coating being provided with a plurality of pits or depressions in its rear surface constituting voids remaining beneath certain of the reinforcing elements.

2. An article of the class described comprising the combination of a rigid cushion coating having reinforcing elements embedded therein adjacent its rearward surface, a surface coating covering and consolidated with said cushion coating and containing waterproofing materials, and reinforcing elements embedded in said coatings at their zone of consolidation, the cushion coating having voids remaining in its rear portion under certain of the reinforcing elements.

3. A structure of the sort specified comprising the combination with a suitably supported scratch coating, of a surface element including a cushion coating laid upon the scratch coating, reinforcing elements embedded in the rearward portion of the cushion coating, a surface coating consolidated with the cushion coating at the front surface thereof and covering the same, reinforcing elements disposed in the cushion and surface coatings in their zone of conjunction, the cushion coating having rearwardly opening pits or depressions and the scratch coating having integral portions thereof extended into said pits or depressions, whereby the surface element is retained against movement on the scratch coating.

4. A structural article of the sort described comprising the combination of a cushion coating having reinforcing elements embedded therein, a surface coating of greater density than the cushion coating covering one surface thereof and consolidated therewith, and reinforcing elements embedded in said coatings in their zone of conjunction.

5. A structural article of the sort described comprising a sheet of coherent material having reinforcing elements embedded therein adjacent its rear surface, said sheet having a plurality of voids therein extending inwardly from its rear surface behind the reinforcing elements and in association therewith, said voids forming locking means for reception of plastic material into the vicinity of the reinforcing elements, whereby to anchor the article in place.

In testimony whereof I have hereunto subscribed my name.

EDWARD N. BIEGLER.